

June 30, 1931.

H. RABEZZANA

1,812,495

ELECTRICAL CONTACT

Filed Jan. 31, 1929



Fig. 1



Fig. 2

Inventor

Hector Rabezzana

By Blackmore, Spence & Blunt

Attorneys

## UNITED STATES PATENT OFFICE

HECTOR RABEZZANA, OF FLINT, MICHIGAN, ASSIGNOR TO A C SPARK PLUG COMPANY,  
OF FLINT, MICHIGAN, A COMPANY OF MICHIGAN

## ELECTRICAL CONTACT

Application filed January 31, 1929. Serial No. 336,470.

This invention relates to contacts such as are employed for switches, make and break devices, relays and the like. Such contacts are subject to rapid deterioration in service as a result of the sparking which takes place particularly when the contact points separate. This sparking continues until the resistance across the air gap which separates the points is higher than the applied voltage. It is well known that to minimize the injurious effects of the spark, it is desirable to shorten its duration as much as possible. For this reason snap-switches are used that open and close the circuit at high speed. Where heavy currents are encountered, magnets are used in an effort to quickly quench the arc. In other cases condensers are employed to reduce sparking.

My invention has to do with greatly reducing the duration of the spark and the injurious effects of sparking by properly selecting and fabricating the materials of which the contacts are made.

It has heretofore been generally accepted that the sparking voltage across the separating contacts and hence the duration of the spark is independent of the material of which the contacts are composed. On the contrary, I have found that the duration of the spark is greatly lengthened by the presence in the contact metal of certain impurities which have heretofore escaped observation, and which markedly affect the sparking voltage. I have found this to be the case even where the impurities are present in such small amounts as to be incapable of detection by chemical analysis.

The impurities to which I refer comprise chemical elements which are characterized by the ease with which they give off electrons. This is often otherwise expressed by stating that the elements have a low work function; that is, that a relatively small amount of work is required to remove an electron from the element. Work function may be measured by measuring the thermo-ionic emission and in various other ways. The class of elements having a low work function are in general electro-positive and include the alkali and alkaline earth metals. Specifically the

group comprises lithium, sodium, potassium, rhubidium, caesium, beryllium, magnesium, calcium, strontium, barium and radium. I have found that the presence in the contacts of any of these elements, whether as elements, alloys, or compounds, even in slight traces, results in a reduction of the sparking voltage and consequently in increased duration of the spark and greater destructive effect. Not only is this the case, but these materials likewise produce a great variation in the sparking voltage from spark to spark since the distribution of the impurities throughout the contact is often not uniform, and since the percentage of the impurities decreases with the increased use of the contact for the reason that the low work function elements leave the contacts at a faster rate than the high work function elements.

According to my invention I so select the contact materials, and so treat them in manufacture as to insure that none of the elements of low work function shall be present even in the smallest amounts. Their presence may be detected by spectroscopic analysis, and by studies of thermo-ionic emission, and in case such analysis should reveal them to be present in objectionable amounts, I may effect their removal by a suitable process such as by "cooking" the contact metal under high vacuum as explained in the following specification.

With substantially all traces of the elements of low work function removed from the contact material, the duration of the sparking will be greatly lessened, and the contacts will have greatly lengthened life with more uniform sparking voltage. This will make it possible to substitute less expensive metals or alloys for the materials now used.

On the drawings I have shown diagrammatically in Figure 1 a pair of contacts made of my improved materials. In Figure 2 I have pictured diagrammatically the process employed for detecting the presence of objectionable materials and removing them from the contact metal.

The contacts illustrated at 2 are of the conventional type used on the interrupters of

55

60

65

70

75

80

85

90

95

100

ignition coils used on automobile engines. However the invention is applicable to all kinds of switches and make and break devices; in other words to all devices designed to effect interruption of an electric circuit.

5 The contacts may be of any desired metals or alloys of metals having a high work function. They must be devoid of any substantial traces of any of the low work function metals. To accomplish this not only requires the utmost care in the selection of the raw materials from which the contact metal is made, but also strict control and even modification of the manufacturing processes involved in reducing the metal, refining it, drawing and forming it, for even the slightest trace of any of the low work function metals or any of their compounds will have an appreciable effect upon the sparking voltage. And in general, throughout the manufacturing process from the raw material to the finished product care must be taken that the undesirable low work function elements are not introduced into the contact metal.

20 25 To insure that contact metal free of low work function elements is obtained, it will be found necessary to test the material preferably by employing the same method of "cooking" under vacuum that may be used to remove the objectionable material when its presence has been ascertained. In many cases mere chemical analysis will not show the presence of the impurities. The preferred method of testing is illustrated in Figure 2, where 3 35 is a vacuum chamber, here shown in the form of a bell jar. Vacuum is maintained by connection at 4 to a pump, not shown, which may be the well known Gaede molecular type. At 6 I have shown a strip of the contact metal 40 connected by suitable conductors to the secondary side of a transformer 8, the primary being connected to a suitable source of power. 10 indicates a plate arranged in parallel with the contact metal 6. In actual practice the 45 contact metal and the plate are arranged as close together as possible to increase the electron flow. The plate is given a positive charge by connection to a storage battery 12, the negative pole of which is connected 50 to the secondary side of the transformer. 14 indicates an ammeter connected in series with the plate 10 and battery.

Upon heating the contact metal 6 to a red heat electrons are given off in quantity 55 and are attracted by the plate 10 because of its positive charge. The amount of electron flow thus produced is measured by the ammeter. By comparison of the ammeter reading with that obtained where pure contact 60 metal is used the amount of undesirable low work function metal may be determined. Should the reading indicate the presence of an undesirably large trace of the metal, it is possible, by using the method described for 65 a sufficient time usually a few hours, to effect

a removal of the major portion of the material, since it leaves the wire at a greater rate than the base metal. When the ammeter reading indicates depletion of the low work function metal, the operation may be stopped, 70 and the metal shaped into the desired form for contacts.

In some cases, little, if any, treatment may be necessary to remove the undesirable elements for the raw materials used may be 75 relatively pure, and the processes of manufacture may be so modified and conducted with such care as to prevent the introduction of the undesirable elements into the contact. However, in most cases, it will be found desirable to test the metal as above indicated prior to employing it for contacts. In other cases, it may be necessary to cook the metal for several hours to remove the undesirable 80 material.

Owing to the higher sparking voltage obtained by the use of contact metals made as described in this specification and the resultant shorter duration of the sparking, it is apparent that my contacts will last much 85 longer than those made by ordinary manufacturing methods. This will, in some cases, permit the substitution of cheaper metals for the more expensive spark resisting metals, such as, platinum, silver, and the like, without 90 decrease in serviceability.

I claim:

1. An electrical contact composed entirely of metal of high work function. 100 2. The method of preparing electrical contacts which consists in reducing the metal or alloy to a condition of relative purity, subjecting it to high vacuum adjacent a positively charged body to indicate the presence of material of low work function, removing 105 said material, and fabricating the contact from the refined material.

3. The method of preparing electrical contacts which consists in reducing the metal or alloy to a condition of relative purity, testing the metal for the presence of elements of low work function, removing the said elements if their presence is indicated, and fabricating the contacts from the metal thus refined. 110

4. The method of preparing high work function metal for use in electrical contacts which consists in removing therefrom all traces of low work function materials. 115

In testimony whereof I affix my signature.

HECTOR RABEZZANA. 120